# EUROPEAN PATENT SPECIFICATION

(11) **EP 1 230 326 B1**
(45) Date of publication and mention of the grant of the patent: **14.06.2006**
(21) Application number: 00974402.0
(22) Date of filing: 17.10.2000
(51) Int. Cl.: C10L 1/04

(54) **Method for depressing the freezing point of a kerosine jet fuel blend**
Verfahren zur Verringerung des Gefrierpunktes eines Kerosin enthaltenden Turbinenbrennstoffs
Procédé de diminution du point de congélation d'un mélange de carburants contenant kérosène

(30) Priority: 29.10.1999 GB 9925640
(43) Date of publication of application: 14.08.2002
(73) Proprietor: ExxonMobil Research and Engineering Company, Annandale, NJ 08801 (US)
(72) Inventor: ASHTON, Simon, Christopher, Peter, Ashtead KT21 2PA (GB)
(74) Representative: Troch, Geneviève
(86) International application number: PCT/EP2000/010186
(87) International publication number: WO 2001/032811

(56) References cited:
- GB-A- 735 134
- US-A- 3 111 482

## Description

This invention relates to jet fuels, especially kerosine based fuels, with improved cold flow properties.

It is well known that liquid hydrocarbons change phase and tend to deposit solid crystals of wax at low, freezing temperatures. However, the nature of the crystals and extent to which deposition occurs depends very much on the molecular structure of the liquid hydrocarbons and their solubility. Thus, the freezing points are usually the highest for high molecular weight n-paraffins, relatively lower for branched chain paraffins and are the lowest for hydrocarbons rich in naphthenes and aromatics. Since the major component of jet fuel come from fractions forming the kerosine boiling range, the amount of high molecular weight n-paraffins in this fraction dictate the freezing point of jet fuels. The components responsible for controlling the freezing point in jet fuels are generally in the high-boiling end of such a fraction. Hence, the final boiling point of the fractions of kerosine which are or can be used as jet fuels is governed by considerations of the freezing point of a given fraction. Most jet fuels are straight-run distillates. The composition of the crude feed being subjected to distillation determines the composition of the fraction boiling within the kerosine boiling range and hence the freezing point of the jet fuel.

Hitherto, in some refineries, some of the aforementioned problems have been mitigated by chemically adjusting the composition of some of these fractions used in jet fuels by processes such as eg hydrocracking. In the latter process, the heavier paraffinic and aromatic fractions are broken down into relatively smaller molecules and are hydrogenated at the same time. This is particularly the case with long-chain paraffins which are cracked into smaller molecules having a molecular weight within the desired range and the process simultaneously results in branched chain molecules being formed. Thus, the process gives rise to products having much lower freezing points than that of the original distillate prior to hydrocracking.

It has also been suggested in EP-A-0282342 that cold-flow properties of fuels can be improved by adding to said fuel a minor proportion of a copolymer of (i) an α-olefin 2-17 carbon atoms per molecule or an aromatic substituted olefin having 8-40 carbon atoms per molecule and (ii) a mono- or a di-alkyl ester selected from fumarates, itaconates, citraconates, mesaconates, trans- or cis-glutaconate in which the alkyl group has 8-23 carbon atoms. However, these are believed not to be adequate to meet proposed and future legislation with respect to freezing points of fuels.

GB 735134 further suggests that the addition of at least 5% by volume of C8 to C9 aromatic hydrocarbons to a major proportion of mineral oil boiling in the range of from 38 to 315°C produces fuel compositions suitable for air craft engines having a reduced tendency to plug the fuel filters at low temperatures.

Whilst the methods currently being used meet the legislation as it stands at present, jet fuels are uniquely likely to be exposed to very low temperatures, especially when flying at high altitudes or when they are on long-haul flights. Other aspects affecting the freezing point of fuels include, flight time, altitude, ambient air temperature, airspeed, fuel pickup temperature, and airframe design which determines the heat transfer characteristics. In the latter context, risk of freezing is also greatest at wing tips, where the highest surface to fuel volume ratio occurs. Under these conditions, the fuel is susceptible to deposition of wax crystals due to insufficiently low freezing points and consequently, may result in problems of pumpability with catastrophic consequences. In order to avoid such incidents, ASTM D2386 has laid down a relationship between the freezing point of jet fuel will still flow can vary from 1-10°C below the freezing point. Thus, this definition is believed to be insufficient, if it becomes necessary for the jets to operate at or near the freezing point. The currently accepted standard according to DEF STAN 91-91/1 is for jet fuels to have a freezing point at or below -47°C, which is considered to be reasonable safe with respect to operational needs.

Furthermore, it is also in the interests of the producers and suppliers of jet fuels to maximize the fraction which can be classed as the kerosine boiling range thereby maximizing the yield of jet fuel that can be obtained by distillation of a given crude oil. The dependency of the yield of the desired jet fuel fraction from a given crude oil varies with the origin of the crude. Hence, freezing point is a usefuel guide for determining whether a given crude is a commercially viable source of straight-run distillates which can be used as jet fuels.

As mentioned previously, various methods have been tried to mitigate the risk of fuels cooling down to deposit wax crystals and thereby making it difficult to pump thereby causing blockage of fuel filters or even, in some instances causing solidification of the fuel in the storage tanks themselves. One such method is, for instance, heating the fuel prior to the LP filter to ensure that the fuel temperature is at least 3°C above the freezing point of the fuel. More recently, use of chemical additives to depress the freezing point of such fuels has also been considered. However, the fuel specification for both civil and military aircraft (as laid down by DEF STAN 91-91) is very stringent and long term testing is needed before any of these can be allowed to be used. For instance, the only fuel containing up to 50% synthetic material and is approved by DEF STAN 91-91-3 is a jet fuel produced by Sasol. Whilst a number of other additives have been allowed, such as eg antioxidants, static dissipators, metal deactivators, lubricity improvers, icing inhibitors and thermal stability improvers, none has been approved hitherto for depressing the freezing point of such fuels.

It has now been found that the freezing point of jet fuels can be depressed well below the minimum levels specified in DEF STAN 91-91/1 by blending therewith a fraction from the distillation process of petroleum crudes.

Accordingly, the present invention relates to a method for depressing the freezing point of a kerosine jet fuel blend to a value lower than -53.5°C by blending a major amount of a kerosine fraction boiling within the range of 140°C to 250°C with 0.5 to 15% by volume of the total blend of naphtha fraction produced by the catalytic cracking of heavy gas oil (hereafter "HCCN") which has a distillation range of T₅ = 165°C to T₉₅ = 210°C and an aromatics content of at least 50% by volume to produce a jet fuel blend having a total aromatic content in the range of from 15 to 25% by volume and a freezing point below that of the kerosine prior to blending.

The kerosine fraction forming the major component of such jet fuel blends suitably has a boiling range of T₅ = 145°C to T₉₅ = 248°C, preferably a range of T₅ = 150°C to T₉₅ = 245°C. The amount of the kerosine fraction in the jet fuel blend of the present invention is suitable greater than 75% by volume, preferably in the range from about 80-99%, more preferably from 85-95% by volume of the total blend comprising the kerosine fraction and the HCCN.

The HCCN is a relatively light fraction derived by catalytic cracking of the so-called gasoil fraction during the refining of petroleum crudes. The catalytic cracking of the gasoil fraction to obtain HCCN can be carried out by any of the known conventional catalytic cracking methods. Such methods are well known in the art and are described in detail for instance by Keith Owen and Trevor Colley in "Automotive Fuels Reference Book", Second Edition, published by the society of Automotive Engineers, Inc, Warrendale, PA, USA (1995). Sepcifically reference is made to Chapter 3 of this textbook at pages 29-49, Chapter 16 at pages 419-469 and 865-890, the latter pages forming Appendix 12 which is a 'Glossary of Terms'. The HCCN fraction is substantially unhydrorefined, ie it has not been subjected to hydrorefining. The HCCN has an aromatic content suitably from 50-75% by volume and preferably from 60-75% by volume. The amount of HCCN required to form such blends is preferably from 2.5 to 10% by volume of the total blend.

The freezing point of such a blend can be determined by a number of methods. This can be done, for instance, by detecting the cloud point of blend using optical sensors or by absorption of light through a sample of the blend. It can also be determined by monitoring the change in cooling rate of the blend as energy is absorbed in the formation of, or released in the dissolution of wax crystals. The latter method can be carried out using a freeze point analyser (Models FPA-30, FPA-50 and FPA-70, marketed by Phase Technology Inc). Alternatively, the freezing point, aromatics and saturated content can be determined using near infra-red (NIR) methods. Yet another method for determining freezing points is the so-called cold-filter plugging point method (hereafter "CFPP"). In another method, known as the Setapoint Detector method (ex Stanhope-Seta), the filter flow of aviation fuels is measured at low temperatures across a stainless steel filter. In this method a sample is subjected to a programmed cooling cycle by water-cooled thermoelectric modules, while a pump maintains an oscillating flow at constant rate across the filter. Separated wax crystals cause an increase in pressure which is sensed electronically. There is also the Institute of Petroleum method (IP 16) of determining freezing points.

The freezing point of the jet fuel blend as determined by the IP 16 method has been found to be well below that of the kerosine fraction in the absence of the HCCN component. For instance, a kerosine fraction without the HCCN component has a freezing point of -53.5°C. HCCN alone has a freezing point of -42 to -45°C. However, the same fraction when blended with 2.5% by volume of HCCN has a freezing point of -54°C, when blended with 5% by volume of HCCN has a freezing point of -54.5°C and when blended with 10% by volume of HCCN has a freezing point of-55°C. Whilst in absolute terms these numbers do not appear significant, in respect of the general risk of waxes crystallising from fuels, these numbers are very significant and reduce the potential risk of blockage of filters and pumps by an order of magnitude. Herein lies the feature of the invention.

A further feature of the present invention is that the HCCN used in the blends to depress the freezing point of jet fuels is substantially a natural component of the petroleum crudes from which the fuel itself is derived. Hence, there are no problems of compatibility problems nor indeed any of the problems associated with external additives.

The method of the present invention may comprise the addition any of the conventional additives used in such fuel compositions. For instance, *inter alia* approved additives such as antioxidants, static dissipators, metal deactivators, lubricity improvers, fuel system icing inhibitors, thermal stability improvers, drag reducing agents, dyes may be added to the blend.

The present invention is further illustrated with reference to the following Examples:

### EXAMPLES:

A kerosine fraction was taken as the base fuel and was blended with various amounts of HCCN and the various properties measured including the freezing points of the each of the two components and the blends thereof. The freezing points were measured according to the standard Institute of Petroleum (IP16) technique.

The tabulated results below show that in spite of the HCCN fraction having a relatively higher freezing point than the base kerosine and in spite of the density of the HCCN fraction being significantly higher than that of the base kerosine, the eventual result of blending the two is to substantially depress the freezing point of the blend to below the value of the base kerosine without adversely affecting the composition of the fuel to any noticeable degree.

| Parameters | Kerosine (%v/v) | HCCN (% v/v) | Amount of HCCN (% v/v) of the total blend with Kerosine | | | |
|---|---|---|---|---|---|---|
| | 100 | 100 | 2.5 | 5.0 | 7.5 | 10 |
| Aromatics (% v/v) | 17.7 | 66.0 | 19.0 | 19.3 | 21.5 | 21.9 |
| Olefins (% v/v) | 0.4 | 3.2 | 0.7 | 0.7 | 0.6 | 0.6 |
| Distillation IBP(°C) | 147.5 | 83.4 | 150.2 | 151 | 151.1 | 149 |
| End Point (°C) | 243.1 | 230.0 | 242.3 | 240.9 | 241.0 | 242.9 |
| Flash Point (°C) | 43.0 | 38.5 | 42.0 | 41.5 | 41.0 | 41.0 |
| Freeze Point(°C) | -53.5 | -44.5 | -54.0 | -54.5 | -55.0 | -55.0 |
| KV₂₀(mm/s) | 3.74 | - | - | - | - | - |
| Density (15°C) | 798.2 | 849.4 | 799.3 | 800.8 | 802.2 | 803.3 |

## Claims

1. A method for depressing the freezing point of a kerosine jet fuel blend to a value lower than -53.5°C, said method comprising blending a major amount of a kerosine fraction boiling within the range of 140° to 250°C with 0.5 to 15 % by volume of the total blend of a naphtha fraction produced by the catalytic cracking of heavy gas oil (HCCN) which has a distillation range of T₅ = 165°C to T₉₅ = 210°C and an aromatics content of at least 50 % by volume to produce a blend having a total aromatic content in the range of from 15 to 25% by volume and a freezing point below that of the kerosine prior to blending.

2. The method according to Claim 1, wherein the kerosine fraction forming the major component of the blend has a boiling range of T₅ = 145°C to T₉₅ = 248°C.

3. The method according to any one of the preceding Claims, wherein the kerosine fraction forming the major component of the blend has a boiling range of T₅ = 150°C to T₉₅ = 245°C.

4. The method according to any one of the preceding Claims, wherein the amount of the kerosine fraction in the jet fuel blend is in the range of 80-99 % by volume of the total blend comprising the kerosine fraction and the HCCN.

5. The method according to any one of the preceding Claims, wherein the HCCN fraction is substantially unhydrorefined and has a boiling range of T₅ = 165°C to T₉₅ = 210°C.

6. The method according to any one of the preceding Claims wherein one or more additives selected from antioxidants, static dissipators, metal deactivators, lubricity improvers, fuel system icing inhibitors, thermal stability improvers, drag reducing agents and/or dyes are added to the blend.

## Patentansprüche

1. Verfahren zum Herabsetzen des Gefrierpunkts eines Kerosindüsentreibstoffgemisches auf einen Wert unter -53,5°C, bei dem eine größere Menge einer im Bereich von 140° bis 250°C siedenden Kerosinfraktion mit 0,5 bis 15 Vol.% des Gesamtgemisches einer Naphthafraktion gemischt wird, die durch katalytisches Cracken von schwerem Gasöl ("HCCN") hergestellt worden ist, einen Destillationsbereich von T₅ = 165°C bis T₉₅ = 210°C und einen Aromatengehalt von mindestens 50 Vol.% hat, um ein Gemisch mit einem Gesamtaromatengehalt im Bereich von 15 bis 25 Vol.% und einem Gefrierpunkt unter demjenigen des Kerosins vor dem Mischen herzustellen.

2. Verfahren nach Anspruch 1, bei dem die Kerosinfraktion, die die Hauptkomponente des Gemisches bildet, einen Siedebereich von T₅ = 145°C bis T₉₅ = 248°C hat.

3. Verfahren nach einem der vorhergehenden Ansprüche, bei dem die Kerosinfraktion, die die Hauptkomponente des Gemisches bildet, einen Siedebereich von T₅ = 150°C bis T₉₅ = 245°C hat.

4. Verfahren nach einem der vorhergehenden Ansprüche, bei dem die Menge der Kerosinfraktion in dem Düsentreibstoffgemisch im Bereich von 80 bis 99 Vol.% des Gesamtgemisches liegt, das die Kerosinfraktion und das HCCN umfasst.

5. Verfahren nach einem der vorhergehenden Ansprüche, bei dem die HCCN-Fraktion im Wesentlichen nicht hydroraffiniert ist und einen Siedebereich von T₅ = 165°C bis T₉₅ = 210°C hat.

6. Verfahren nach einem der vorhergehenden Ansprüche, bei dem ein oder mehrere Additive ausgewählt aus Antioxidantien, Zerstreuungsmitteln für statische Ladung, Metalldeaktivatoren, Schmierfähigkeitsverbesserern, Treibstoffsystemvereisungsinhibitoren, Wärmebeständigkeitsverbesserern, Stirnwiderstandsverringerungsmitteln und/oder Farbstoffen zu dem Gemisch gegeben werden.

## Revendications

1. Procédé pour abaisser le point de congélation d'un mélange de carburant contenant du kérosène à une valeur inférieure à -53,5° C, ledit procédé consistant à mélanger une quantité principale d'une fraction de kérosène bouillant dans la gamme de 140° C à 250° C avec 0,5 à 15 % en volume du mélange total d'une fraction de naphta produite par le craquage catalytique de gasoil lourd (HCCN) qui a une gamme de distillation de T₅ = 165° C à T₉₅ = 210° C et une teneur en composés aromatiques d'au moins 50 % en volume pour produire un mélange ayant une teneur totale en composés aromatiques dans la gamme de 15 % à 25 % en volume et un point de congélation en dessous de celui du kérosène avant le mélange.

2. Procédé selon la revendication 1, dans lequel la fraction de kérosène formant le composant principal du mélange a une gamme d'ébullition de T₅ =145° C à T₉₅ = 248° C.

3. Procédé selon l'une quelconque des revendications précédentes, dans lequel la fraction de kérosène formant le composant principal du mélange a une gamme d'ébullition de T₅ = 150° C à T₉₅ = 245° C.

4. Procédé selon l'une quelconque des revendications précédentes, dans lequel la quantité de la fraction de kérosène dans le mélange de carburant se situe dans la gamme de 80-99 % en volume du mélange total comprenant la fraction de kérosène et le HCCN.

5. Procédé selon l'une quelconque des revendications précédentes, dans lequel la fraction HCCN est essentiellement non hydro-raffinée et a une gamme d'ébullition de T₅ = 165° C à T₉₅ = 210° C.

6. Procédé selon l'une quelconque des revendications précédentes, dans lequel on ajoute au mélange un ou plusieurs additifs choisis parmi les antioxydants, les dissipateurs statiques, les désactivateurs de métaux, les agents améliorant le pouvoir lubrifiant, les inhibiteurs de formation de glace du système de carburant, les agents améliorant la stabilité thermique, les agents réduisant la traînée et/ou les colorants.
